



US006440896B1

(12) **United States Patent**  
Szajewski et al.

(10) **Patent No.:** US 6,440,896 B1  
(45) **Date of Patent:** Aug. 27, 2002

(54) **IMAGING MEMBER WITH  
MULTIFUNCTIONAL COUPLER AND  
OXIDANT**

(75) Inventors: **Richard P. Szajewski; Lyn M. Irving**,  
both of Rochester, NY (US)

(73) Assignee: **Eastman Kodak Company**, Rochester,  
NY (US)

(\*) Notice: Subject to any disclaimer, the term of this  
patent is extended or adjusted under 35  
U.S.C. 154(b) by 0 days.

(21) Appl. No.: **09/162,083**

(22) Filed: **Sep. 28, 1998**

(51) **Int. Cl.<sup>7</sup>** ..... **B41M 5/136**

(52) **U.S. Cl.** ..... **503/201**; 347/105; 428/195;  
503/202; 503/204; 503/210; 503/211; 503/216

(58) **Field of Search** ..... 347/105; 428/195;  
503/201, 212, 202, 204, 210, 211, 216

(56) **References Cited**

U.S. PATENT DOCUMENTS

|             |           |                  |       |         |
|-------------|-----------|------------------|-------|---------|
| 3,906,141 A | 9/1975    | Anderson et al.  | ..... | 428/411 |
| 4,266,229 A | 5/1981    | Mansukhani       | ..... | 346/11  |
| 5,501,150 A | 3/1996    | Leenders et al.  | ..... | 101/466 |
| 5,568,173 A | 10/1996   | Leenders et al.  | ..... | 347/96  |
| 5,621,448 A | 4/1997    | Oelbrandt et al. | ..... | 347/96  |
| 5,621,449 A | 4/1997    | Leenders et al.  | ..... | 347/101 |
| 6,143,693 A | * 11/2000 | Irving et al.    | ..... | 503/201 |

6,197,722 B1 \* 3/2001 Irving et al. .... 503/201

OTHER PUBLICATIONS

Theory of the Photographic Process, 4th Ed. James, 1977, pp  
291-373.

Anonymous, Digital Silver in Digital Pro, pp 6-8, 1997.

Sambucetti et al., IBM Technical Disclosure Bulletin, vol.  
20 pp 5423-4, 1978.

Pimbley, IBM Technical Disclosure Bulletin, vol. 23, p.  
1387, 1980.

\* cited by examiner

*Primary Examiner*—Bruce H. Hess

(74) *Attorney, Agent, or Firm*—Paul A. Leipold; Lynne M.  
Blank

(57) **ABSTRACT**

The invention relates to an imaging member comprising at  
least one light insensitive layer comprising an oxidant and a  
multifunctional dye-forming coupler. It further relates to a  
method of imaging comprising providing an imaging mem-  
ber comprising at least one light insensitive layer comprising  
a catalytic center and multifunctional dye-forming coupler,  
imaginewise applying a first developer solution that will react  
with said multifunctional dye-forming coupler, imaginewise  
applying a second developer solution that will react with  
multifunctional dye-forming coupler, wherein said first  
developer solution and said second developer solution pro-  
duce different colors.

**65 Claims, No Drawings**

**IMAGING MEMBER WITH  
MULTIFUNCTIONAL COUPLER AND  
OXIDANT**

**FIELD OF THE INVENTION**

This invention relates to an imaging member comprising at least one light insensitive layer comprising an oxidant and a multifunctional dye forming coupler. It further relates to a method of imaging comprising imagewise applying to such a member distinct developer solutions that will react with said multifunctional dye forming coupler to produce dyes of different colors.

**BACKGROUND OF THE INVENTION**

It has become quite popular to form images on plain or treated papers by the imagewise deposition of inks. This deposition can take place by means of contact or impact printing, as in a printing press or typewriter like arrangement or by a variety of more modern non-impact printing systems. One of these non-impact printing systems is known as ink jet printing.

In ink jet printing, tiny droplets of ink are projected directly onto a receptor surface for printing without physical contact between the printing device and the receptor. The placement of each drop on the printing substrate is controlled electronically. Printing is accomplished by moving the printhead across the paper, or by moving the paper across the printhead.

Different types of ink jet printing are known. Two major forms of ink jet printing are "drop-on-demand" printing and "continuous jet" printing. Continuous jet printing is characterized by pressure-projecting inks through a nozzle to generate drops of ink directed in a continuous stream towards the ink receiving element while passing through an imagewise modulated ink deflection system, thereby allowing ink droplets of the stream to deposit imagewise on the recording element. Drop-on-demand or impulse ink jet differs from continuous ink jet in that the ink supply is maintained at or near atmospheric pressure. An ink drop is ejected from a nozzle only on demand when controlled excitation coming from pressure generated by a piezoelectric element or from pressure generated by local electrothermal evaporation of liquid (thermal bubble jet) is applied to an ink filled channel ending in a nozzle. Acoustic, microfluidic, and electrostatic driven drop-on-demand techniques are also known. These technologies are described in detail by J. L. Johnson, *Principles of Non-Impact Printing*, Palatino Press, Irvine, Calif. (1986), and in *Nebblette's Imaging Processes and Materials*, Eighth Edition, J. Sturges Ed. Van Nostrand, New York, (1989).

When several ink streams are independently employed to imagewise deliver colored inks to a surface, color images can be obtained. The inks employed for this purpose typically fall into one of two categories, pigmented inks and soluble inks. The pigmented inks have the advantage of providing stable color images but are lacking in that the pigment particles rest at the surface of the receiving element and are especially prone to mechanically induced smear and rub-off. Additionally, heads delivering the pigmented inks are prone to clogging. The soluble inks solve the rub-off and clogging problems but suffer in that they are prone to fading and to image smearing in humid environs or when the receiving element is hand handled or otherwise wetted.

In related art, Oelbrandt et al in U.S. Pat. No. 5,621,448 describes the imagewise application of a reducing agent solution to a receiving element having a reducible silver salt to imagewise form a metallic silver image. The possibility of intensifying this black image by the presence of color coupler dyes is mentioned. Sambucetti and Seitz, in IBM

Technical Disclosure Bulletin vol. 20, pages 5423-4 (1978) describe the formation of images by imagewise applying a jet or mist of a reactive species to a paper impregnated with a reactant to again form metallic images. Leenders et al in U.S. Pat. No. 5,621,449 describes imagewise applying a reducing agent to a receiver element comprising a reducible silver salt to form a metallic silver image. The possibility of intensifying this black image by the presence of color coupler dyes is mentioned. The methods described by these workers are directed at providing black images which, in some cases, may be intensified by the presence of color couplers. These methods all suffer in that the receiving element or the imagewise mist must contain between them sufficient developing agent and metal salts to form a dense image, thus requiring that large quantities of solution be employed to deliver the components. The element dries slowly and forms only a black-and-white image at best. Pimbley, in IBM Technical Disclosure Bulletin vol. 23, pages 1387 (1980) discloses that leuco dyes or vat dyes can be applied to a paper coated or impregnated with an oxidizing agent. This method suffers in that the leuco or vat dyes are unstable and thus leads to a material having poor shelf life. Sufficient details to practice this disclosure are not revealed.

**PROBLEM TO BE SOLVED BY THE  
INVENTION**

There remains a need for a method of imaging that has the convenience of ink jet but with performance and smear resistance like that obtained with photographic images.

**SUMMARY OF THE INVENTION**

It is an object of this invention to provide an imaging member that has excellent raw stock and storage stability.

It is a further object of this invention to provide an imaging member that enables the production of viewable images having excellent color saturation and color gamut.

It is another object of the invention to provide an imaging member that enables the production of viewable color images having excellent resistance to dark and light fade, as well as resistance to image smear and rub-off.

It is yet another object of this invention to provide an imaging member that enables the production of viewable color images with good resistance to moisture and humidity.

It is yet a further object to provide a method of image formation which results in colorful and stable images that are resistant to dark and light fade, not susceptible to image smear and rub-off, and stable to moisture and humidity.

It is also an object of this invention to provide a method of image formation that alleviates the problem of head clogging.

These and other objects of the invention are accomplished by providing an imaging member comprising at least one light insensitive layer comprising an oxidant and a multifunctional dye forming coupler. The objects of the invention are further accomplished by providing a method of imaging comprising providing an imaging member comprising at least one light insensitive layer comprising an oxidant and a multifunctional dye forming coupler, imagewise applying a first developer solution that will react with said multifunctional dye forming coupler, imagewise applying a second developer solution that will react with multifunctional dye forming coupler, wherein said first developer solution and said second developer solution produce different colors.

**ADVANTAGEOUS EFFECT OF THE  
INVENTION**

This invention provides simple and fast printing of images with photographic image stability and color.

## DETAILED DESCRIPTION OF THE INVENTION

The invention has numerous advantages. The imaging member of the invention shows excellent raw stock stability, and images formed using the member show excellent resistance to dark and light fade, are insensitive to moisture, temperature and humidity, and show excellent resistance to image smear and rub-off. Further, the color images show high saturation and excellent color gamut. The method of providing images is simple, fast, and easy to operate. Additionally, both the material and the method are compatible with a variety of solution application apparatus, thus making the material and method of great value to those already owning digitally addressable solution application printers. By incorporating a stable photographic coupler within a protective medium to form an imaging member and imagewise applying a series of distinct photographic coupling developers to that member, dyes of exceptional stability and colorfulness can be formed in an imagewise manner. Since the dyes are formed in a protected environment, the problems of image smear and rub-off are alleviated. The photographic dyes formed are especially stable against dark, light, and humidity induced fade. Since the dyes are ballasted, they are also resistant to moisture and humidity induced image smear. By providing the dye forming agents in soluble form, the problems associated with head clogging typically encountered with particulate dyes and pigmented inks are avoided. These and other advantages will be apparent from the detailed description below.

The imaging member of the invention comprises at least one light insensitive layer comprising an oxidant and a multifunctional dye forming coupler. This light insensitive layer is the locus of image formation and is also referred to as an imaging layer. In one embodiment, the light insensitive layer comprises a homogeneous admixture of oxidant and multifunctional dye forming coupler. In another embodiment, the light insensitive layer is itself formed from two or more homogeneous sub-layers which differ in composition. In this latter case, one sub layer can be rich in oxidant, while another can be rich in multifunctional dye forming coupler. When sub layers are employed, they can be adjacent or separated by interlayers. Distinct sub layers can alternatively comprise differing concentrations of oxidant or of multifunctional dye forming coupler so as to enable overall concentration gradients in each of these components. Different sub layers can contain a common multifunctional dye forming coupler and a common oxidant. Alternatively, distinct multifunctional dye forming couplers and oxidant can be employed in one light insensitive layer or in more than one layer or sub layer. The imaging member is preferably light insensitive.

The imaging member can additionally comprise a support which can be a reflective support or a transparent support. When reflective, the support is generally white. When transparent, the support is generally clear, although it can be tinted. Details of support construction are well known in the paper and photographic arts. Particular photographic supports especially useful in this invention, including subbing layers to enhance adhesion, are disclosed in *Research Disclosure*, published by Kenneth Mason Publications, Ltd., Dudley house, 12 North Street, Emsworth, Hampshire PO10 7DQ, England. Vol. 389, September 1996, Item 38957, XV. Supports. In another embodiment, the member can comprise a peelable support and an adhesion layer enabling a formed image to be applied to an object as, for example, to form a customized decorative item. The support can be supplied in roll or sheet form. Alternatively, the support can be a rigid member. In one embodiment, an imaging layer can be located on only one side of the support. In another embodiment, imaging layers can be located on both sides of

the support to provide for double sided images, ease of use, and anticurl properties. In yet another embodiment, the imaging layer and the support can form an integral unit. In this embodiment, the support itself can function as a vehicle for the multifunctional dye forming coupler and the oxidant. When the imaging layer differs in composition from the support, it will generally be between 1 and 50  $\mu\text{m}$  in thickness. Preferably, it will be between 2 and 40  $\mu\text{m}$  in thickness. More preferably, it will be between 3 and 30  $\mu\text{m}$  in thickness.

TABLE 1

| Imaging Member<br>Support |
|---------------------------|
|---------------------------|

Table 1 shows, in schematic form, an embodiment of an imaging member of the invention. This embodiment comprises an imaging layer coated on a support. The imaging layer comprises the multifunctional coupler and oxidant in a vehicle. In the Table 1 embodiment, the developers or developer precursors are individually applied imagewise to the imaging layer. The member can be optionally heated in an imagewise or non-imagewise manner to speed the process and promote drying. The oxidant reacts with the imagewise applied developers or developer precursors to form the oxidized form of the developers or developer precursors and a reduced form of the oxidant. The oxidized form of the developer or developer precursor, in turn, reacts with the multifunctional dye forming coupler to form dye deposits in an imagewise fashion relative to the position at which the developer or developer precursor was initially applied. In this way a viewable image is formed.

By way of illustration, a transparent support is coated with a hardened gelatin layer comprising 1-phenyl-3-benzamido-5-pyrazolone in a hydrocarbon coupler solvent along with silver behenate, and this in turn is overcoated with a protective hydrophilic colloidal layer. A solution of 4-N,N-diethyl-2,6-dimethylphenylenediamine is applied in an imagewise fashion, and an imagewise cyan dye deposit is formed. A solution of 4-N,N-diethyl-2-tert-butyphenylenediamine is applied in an imagewise fashion, and an imagewise magenta dye deposit is formed. A solution of 2-chloro-4-N,N-diethylphenylenediamine is applied in an imagewise fashion, and an imagewise yellow dye deposit is formed, thus together forming a full color image which can be directly viewed, projected, or backlit.

By way of further illustration of a distinct embodiment, a paper is impregnated with 1-phenyl-3-methyl-5-pyrazolone in the presence of 1,4-cyclohexyldimethylene bis(2-ethylhexanoate) and silver benzotriazole. A solution of 4-N,N-diethyl-2,6-dimethylphenylenediamine is applied in an imagewise fashion, and an imagewise cyan dye deposit is formed. A solution of 4-amino-2,6-dichlorophenol is applied in an imagewise fashion, and an imagewise magenta dye deposit is formed. A solution of 4-N-phenylenediamine is applied in an imagewise fashion, and an imagewise yellow dye deposit is formed, thus together forming a full color image suitable for direct viewing.

In illustration of yet another embodiment, both sides of a reflective support are coated with a subbing layer, then coated with a hydrophilic colloidal layer containing coupler A-7 whose structure is shown below, admixed with silver 5-amino-2-benzylthiobenzotriazole, followed by a protective overcoat layer having a UV absorber. A solution of 4-(N-ethyl-N-2-methanesulfonylaminooethyl)-2,6-dimethylphenylenediamine is applied in an imagewise fashion, and a cyan dye deposit is formed. A solution of 4,5-dicyano-2-isopropylsulfonylhydrazino benzene is applied in an imagewise fashion, and an imagewise magenta

dye deposit is formed. A solution 4-hydrazinobenzoic acid is applied in an imagewise fashion, and an imagewise yellow dye deposit is formed. In this way a full color image is formed. The same solutions are then applied in a different imagewise fashion to the opposite side of the member, and a second image is formed. In this way, a two-sided viewable color image is formed.

The imaging member may additionally comprise an overcoat layer that provides for the physical protection of the light insensitive layer before, during, or after image formation. An overcoat layer provides a convenient location for incorporation of addenda that are most effective at or near the surface of the member. The overcoat may be divided into a surface layer and one or more interlayer, the interlayer functioning as a spacer layer between addenda in the surface layer and the imaging layer. In a common variant form, addenda are distributed between the surface layer, any interlayer and the imaging layer with the positioning of the addenda dictated by compatibility of the addenda with the intended function of each layer. These addenda are typically agents which aid in the manufacture and preparation of the imaging member, and in the stability of the imaging member before, during, and after image formation. Typical addenda include but are not limited to coating aids, plasticizers, lubricants, antistats, anti-matting agents, stabilizers, gloss promoting agents, and ultraviolet light absorbers, all as known in the photographic and papermaking arts. Wicking layers which serve to segregate moisture can further be employed. These layer structures and addenda are well known in the art and are disclosed, *inter alia* at *Research Disclosure*, Item 38957, and at *Research Disclosure*, Item 37038 (1995), Section VI, Polymeric Addenda, Section VII, Structure of Stabilizers, Section X, UV Stabilizers, and Section XI, Surfactants, the disclosures of which are incorporated by reference.

The light insensitive layer will generally comprise a vehicle chosen to allow admission of color developer in an imagewise manner. When the color developer is supplied in an aqueous state, the vehicle will be adequately water permeable so as to accept the color developer solution. Any vehicle known in the art which has the requisite properties can be employed for this purpose. Most generally, this will be a hydrophilic colloidal material. In one embodiment the hydrophilic colloidal material can be gelatin or a modified gelatin, such as acetylated gelatin, phthalated gelatin, or oxidized gelatin. Alternatively, the hydrophilic colloidal material can be another water soluble polymer or copolymer including, but not limited to, poly(vinyl alcohol), partially hydrolyzed poly(vinylacetate/vinylalcohol), hydroxy cellulose, poly(acrylic acid), poly(1-vinylpyrrolidinone), poly(sodium styrene sulfonate), poly(2-acrylamido-2-methane sulfonic acid), and polyacrylamide. Copolymers of these polymers with hydrophobic monomers can also be employed. These hydrophilic colloidal materials can be employed alone or in admixture with other hydrophilic colloidal materials. When the member comprises sub layers, overcoats, or such, the vehicle employed in each of these various layers can be the same or can differ so as to provide improved properties. The vehicle can be cross-linked or hardened, all as disclosed in *Research Disclosure*, Item 38957, already cited. Alternatively, non-aqueous color developer solutions and hydrophobic vehicles permeable to these solutions can be employed and are specifically contemplated. The vehicle can be colorless or tinted. When the vehicle is colorless, this means that the optical density of the vehicle in the visible region, i.e., between 400 and 700 nm, is up to 0.2, is preferable up to 0.1, and more preferable up to 0.05.

Any oxidant known in the art which enables the oxidation of the reduced form of a color coupling color developer or

its precursor to its oxidized form can be employed in the practice of this invention. The quantity of oxidant which may be most effectively employed is dictated by the stoichiometry of the coupling reaction, that is, by the stoichiometry of the reaction between the multifunctional dye forming coupler and oxidized developer. Typically two electron-mole equivalents of oxidant are required to oxidize one mole of a two electron mole equivalent developer, that is, a 2-equivalent developer, to its oxidized form. When one mole of a 2-equivalent multifunctional dye forming coupler is employed, these two-electron mole equivalents of oxidant, embedded in the oxidized developer, enable the formation of one mole of dye by a coupling reaction. Alternatively, when one mole of a 4-equivalent multifunctional dye forming coupler is employed with a 2-equivalent developer, then four electron-mole equivalents of oxidant and two moles of developer are required for the formation of one mole of dye. In this later situation, the reaction of one mole of a 4-equivalent multifunctional dye-forming coupler with two moles of oxidized developer results in the formation of one mole of dye, along with the regeneration of one mole of 2-equivalent developer. Although the regenerated developer can be reemployed in a cyclic fashion, thus minimizing the quantity of excess developer present after all of the oxidant has been expended, this later situation is less preferred since any excess developer can eventually lead to the production of unwanted image dye. Preferably, the electron equivalency of the developer and the electron equivalency of the multifunctional dye-forming coupler are equal. While any useful molar ratio of multifunctional dye-forming coupler, developer, and oxidant may be employed, preferably about two electron-mole equivalents of oxidant are employed in combination with about one mole of a 2-equivalent developer and about one mole of 2-equivalent multifunctional dye forming coupler to form maximum density in the practice of this invention. In another embodiment, about four electron-mole equivalents of oxidant are employed in combination with about two moles of a 2-equivalent developer and about one mole of 4-equivalent multifunctional dye forming coupler to form maximum density in the practice of this invention. These optimal ratios can be adjusted to compensate for any inefficacy in the underlying reactions. Practically, the molar ratio of oxidant, counted as electrons, to 2-equivalent multifunctional dye-forming coupler is about 2:1. Preferably the molar ratio of oxidant, counted as electrons, to 2-equivalent multifunctional dye-forming coupler is between about 1.8:1 and 3:1. Likewise, the molar ratio of oxidant, counted as electrons, to 4-equivalent multifunctional dye-forming coupler is about 4:1. Preferably the molar ratio of oxidant, counted as electrons, to 4-equivalent multifunctional dye-forming coupler is between about 3.6:1 and 6:1.

In one embodiment, the oxidant employed is a metal salt which forms metallic deposits on its reduction. Examples of such metal salts include the salts of vanadium, chromium, manganese, iron, cobalt, nickel, copper, niobium, molybdenum, ruthenium, rhodium, palladium, silver, cadmium, tantalum, tungsten, rhenium, osmium, iridium, platinum, and gold. In a preferred embodiment, the metal salt can be chosen from the reducible silver fatty acid salts, the reducible salts of silver alkylacetylide, the reducible salts of silver arylacetylide, the reducible salts of silver alkylamines, the reducible salts of silver arylamines, the reducible salts of heterocyclic silver mercaptides, and the reducible salts of heterocyclic silver thiones. In a particularly preferred embodiment, the metal salt is silver behenate, silver benzotriazole, silver acetylidyne, or silver 5-amino-2-benzylthiobenzotriazole.

In another embodiment, the oxidant employed is a metal salt which can oxidize the applied developers without itself being fully reduced to a metallic form. This embodiment is

advantageous since it leads to an imaging member which forms images lacking in an overall tint caused by reduced metal deposits. Metal salts of metals chosen from Group VA, Group VIA, Group VIIA, Group VIIIA, and Group IB of the periodic table of the elements can be employed in this regard. Examples of such metal salts include, but are not limited to, the higher oxidation state complexes of vanadium, chromium, manganese, iron, cobalt, nickel, copper, niobium, molybdenum, ruthenium, rhodium, palladium, silver, cadmium, tantalum, tungsten, rhenium, osmium, iridium, platinum, and gold.

When a metal salt is employed, the metal salt will generally be of a size and optical density so as not to interfere with viewing of images borne by the imaging member. The metal salt can be atomic, molecular, or particulate in nature. When the metal salt is particulate, it typically has a particle size of up to  $30\text{ }\mu\text{m}$ , preferably of up to  $10\text{ }\mu\text{m}$ , and more preferably of up to  $3\text{ }\mu\text{m}$ . The particles can generally have a size of at least  $0.1\text{ }\mu\text{m}$  and preferably of at least  $0.5\text{ }\mu\text{m}$ . The metal salt can be incorporated in the imaging member in any manner known in the art. When the metal salt is a soluble species, it can be incorporated by solution in the member at manufacture. When the metal salt is particulate, it will typically be incorporated as such in the member at manufacture. Alternatively, the metal salt can be applied to a member prior to, during, or immediately after the application of the developer solution, thereby forming the inventive member in situ. It is preferred that the metal salt be applied to the member at between about 0.2 and 3  $\text{g}/\text{m}^2$ . It is more preferred that the metal salt be applied to the member at between about 0.5 and 2.5  $\text{g}/\text{m}^2$ . The minimum quantity of metal salt required is dictated by the efficiency of dye formation and by the extinction coefficient of the formed dyes. When the reducible metal salt forms metallic particle on reduction, the quantity of metal salt employed should be held as close as possible to this minimum quantity so as to avoid the formation of excess density from metallic particles which can be formed in the imaging member.

In a preferred embodiment, the reducible metal salt chosen is one which can be air oxidized from its reduced form to a more highly oxidized form which is colorless in this more oxidized form. In yet another preferred embodiment, the reducible metal salt chosen is one which is colorless in its reduced form. Such metal salts are well known in the art. These metal salts are especially useful in this invention since highly colored images of improved gamut and hue can be formed in this way.

In another embodiment, a non-metallic oxidant can be employed. The non-metallic oxidant can be incorporated in the member, it can be incorporated in the imagewise applied developer solutions, it can be separately applied, or reliance can be placed on adventitious oxygen. Better stability can be attained by applying the oxidant as a separate solution. Any oxidant useful for cross-oxidizing the developers or developer precursors can be employed. Preferably, the oxidant is a peracid oxidant or its salt. Typical peracid oxidants useful in the practice of this invention include the hydrogen, alkali and alkali earth salts of persulfate, peroxide, perborate, and percarbonate, oxygen, and the related perhalogen oxidants such as hydrogen, alkali, and alkali earth salts of chlorate, bromate, iodate, perchlorate, perbromate, and metaperiodate. Hydrogen peroxide solution is the preferred oxidant. When applied in a less than fully imagewise fashion, the oxidant can serve the dual function of not only oxidizing the imagewise applied developer or developer precursor, but also acting to whiten the member in areas lacking developer or developer precursor, thus providing for improved gamut and brighter colors.

When the oxidant is applied in a solution, the pH of the solution can be pre-adjusted for optimum cross-oxidation as

known in the art, or it can be pre-adjusted for optimum storage stability, with final pH adjustment supplied by the developer solution. The pH adjustment can employ a buffer consisting of an organic or inorganic acid or base and/or a salt thereof. Useful examples include phosphoric acid and salts of phosphates, citric acid and salts of citrate, boric acid and salts of borate or metaborate, acetic acid and salts of acetate, amines and amine salts, urea derivatives and their salts, and ammonium hydroxide. Oxidant stabilizers can be present in an oxidant solution as known in the art. Additionally, the oxidant can be supplied in a blocked form which unblocks and releases the oxidant. When the oxidant is supplied from an oxidant solution, the oxidant will preferably be present in the oxidant solution at a concentration between about 1 and 100  $\text{g}/\text{L}$ . It is more preferred that the oxidant will be present in the oxidant solution at a concentration between about 2 and 50  $\text{g}/\text{L}$ .

When a non-metallic oxidant is employed, a catalyst for cross oxidation can be employed to speed the oxidation of the applied color developer. The catalytic center comprises a metal or metal salt. Any metal or metal salt known in the art which enables the oxidation of the reduced form of a color coupling color developer or its precursor by an oxidant can be employed for this purpose. Examples such metals and metal salts include those chosen from the Group VIIA and Group IB metals and their salts. Specific examples include the metallic deposits of and salts of iron, cobalt, nickel, rhodium, iridium, silver, gold, platinum, palladium, ruthenium, osmium, and copper. In a preferred embodiment, the metal is Carey Lea silver. The catalytic center will generally be of a size and optical density so as not to interfere with viewing of images borne by the imaging member. The catalytic center can be atomic, molecular, or particulate in nature. When the catalytic center is particulate, it typically has a particle size of up to  $5\text{ }\mu\text{m}$ , and preferably has a particle size of up to  $1\text{ }\mu\text{m}$ , and more preferably has a particle size of up to  $0.1\text{ }\mu\text{m}$ . Specific catalytic center materials are preferable selected from the group consisting of deposits of silver, gold, copper, and iron in metallic or salt form. The catalytic center can be incorporated in the imaging member in any manner known in the art. When the catalytic center is a soluble species, it can be incorporated by solution in the member at manufacture. When the catalytic center is particulate, it can typically be incorporated as such in the member at manufacture. Alternatively, the catalytic center can be applied to a member prior to, during, or immediately after the application of the developer solution. While the metal or metal salt forming the catalytic center can be employed in any useful quantity, it is preferably employed in trace amounts. It is preferred that the catalytic center be applied to the member at between about 0.01 and 50  $\text{mg}/\text{m}^2$ . It is more preferred that the catalytic center be applied to the member at between about 0.1 and 10  $\text{mg}/\text{m}^2$ .

Mixtures of the described oxidants can be employed to better form the desired images.

The multifunctional dye forming coupler can be any known coupler that possesses the requisite property of forming different color dyes with the oxidized forms of distinct color developers. Most generally, such a coupler will have structure I:



wherein:

C is a carbon atom at which coupling occurs;

L represents a hydrogen atom or a leaving group covalently bound to C and which is displaced on coupling;

H is an acidic hydrogen atom serving to direct coupling to C and which is covalently bound to C directly or by conjugation; and

Z represents the remainder of the atoms of the coupler, in cyclic or acyclic form, which together provide sufficient electron withdrawal to render H acidic and together provide sufficient ballast function to render the dye formed from the coupler immobile.

When L is H, then the multifunctional dye-forming coupler is 4-equivalent multifunctional dye-forming coupler.

When L is a leaving group which is displaced on coupling, then the multifunctional dye-forming coupler is 2-equivalent

(i) multifunctional dye-forming coupler. It is preferred that L be a leaving group since 2-equivalent multifunctional dye-forming couplers are preferred in the practice of this invention.

5 The coupler I can be monomeric or polymeric in nature. Couplers useful in the practice of this invention are described in *Research Disclosure*, Item 38957, Section X. Dye Image Formers and Modifiers, in *Research Disclosure*, Item 37038 (1995), in Katz and Fogel, *Photographic Analysis*, Morgan & Morgan, Hastings-on-Hudson, New York, 1971, in the Appendix, in Lau et al U.S. Pat. No. 5,670,302 and in European Patent Application EP 0 762 201 A1, the disclosures of which are all incorporated by reference.

15 In a preferred embodiment, the coupler is a pyrazole, a pyrazolone, a pyrazolotriazole, pyrazolotetrazole, a 2-acylamino- 1-naphthol, or a cyanoacetate coupler. Examples of these useful couplers are illustrated in the references cited above. Additional specific examples of these useful couplers are shown as structures M-1 through M-17 of pages 82-83, and as "Coupler 3" of page 98, right column; "Coupler 4", "Coupler 5", "Coupler 8", and "Coupler 9" of page 99, right column; "Coupler 3" of page 100, right column; and "Coupler 4" and "Coupler 5" of page 101, left column in *Research Disclosure*, Item 37038 (1995).

20 25 Specific preferred multifunctional dye forming couplers include but are not limited to the following couplers:

A-1



A-2



11

12

-continued

A-3



A-5

A-4



**13****14**

-continued

A-6

A-7





-continued



Mixtures of multiple multifunctional dye-forming couplers and mixtures of multifunctional dye-forming couplers and other known couplers can be employed in the practice of this invention

The multifunctional dye forming couplers useful in the invention can be incorporated in the imaging member in any manner known in the art. These methods include but are not limited to incorporation as oil-in-water emulsions, known colloquially in the photographic arts as "dispersions", as reverse phase emulsion, as solid particle dispersions, as multiphase dispersions, as molecular dispersions or "Fisher" dispersions, or as polymer loaded dispersions or loaded latex dispersions. When the multifunctional dye forming couplers are polymeric in nature, they can additionally be incorporated merely by physically diluting the polymeric coupler with vehicle. While the multifunctional dye forming coupler can be employed in the member at any concentration that enables the desired formation of a multicolor image, it is preferred that the multifunctional dye forming coupler be applied to the member at between about 50 and 3000 mg/m<sup>2</sup>. It is more preferred that the multifunctional dye forming coupler be applied to the member at between about 200 and 800 mg/m<sup>2</sup>.

The imaging member can further comprise an incorporated solvent. In one embodiment the multifunctional dye forming coupler is provided as an emulsion in such a solvent. In this embodiment, any of the high boiling organic solvents known in the photographic arts as "coupler solvents" can be employed. In this situation, the solvent acts as a manufacturing aid. Alternatively, the solvent can be incorporated separately. In both situations, the solvent can further function as a hue shifter, a coupler stabilizer, a dye stabilizer, a reactivity enhancer or moderator, or as a hue shifting agent, all as known in the photographic arts. Additionally auxiliary solvents can be employed to aid dissolution of the multifunctional dye forming coupler in the coupler solvent. Particulars of coupler solvents and their use are described in the aforesaid mentioned references and at *Research Disclosure*, Item 37038 (1995), Section IX, Solvents, and Section XI, Surfactants, incorporated herein by reference. Specifically useful coupler solvents include but are not limited to tritoluyl phosphate, dibutyl phthalate, N,N-diethyldodecanamide, N,N-dibutyldecanamide, tris(2-ethylhexyl)phosphate, acetyl tributyl citrate, 2,4-di-tert-pentylphenol, 2-(2-butoxyethoxy)ethyl acetate, and 1,4-cyclohexyldimethylene bis(2-ethylhexanoate). The choice of coupler solvent and vehicle can influence the hue of dyes formed as disclosed by Merkel et al in U.S. Pat. Nos. 4,808,502 and 4,973,535. Most generally it is found that materials with a hydrogen bond donating ability can shift dyes bathochromically, while materials with a hydrogen bond accepting ability can shift dyes hypsochromically. Additionally, use of materials with low polarizability can of itself promote hypsochromic dye hue shifts as well as promote dye aggregation. It is recognized that coupler ballasts often enable dyes and dye-coupler mixtures to function as self-solvents with a concomitant shift in hue. The polarizability, and the hydrogen bond donating and accepting ability of various materials, are described by Kamlet et al in *J. Org. Chem.*, 48, 2877-87 (1983), the disclosures of which are incorporated by reference.

Generally two or more distinct developers or developer precursors are employed in the practice of this invention. These developers can be any developers known in the art that are coupling developers and enable the formation of distinctly colored dyes from the same coupler. By distinctly colored is meant that the dyes formed differ in the wavelength of maximum adsorption by at least 50 nm. It is preferred that these dyes differ in the maximum adsorption wavelength by at least 65 nm and more preferred that they differ in the maximum adsorption wavelength by at least 80

nm. It is further preferred that at least a cyan and a magenta, or a cyan and a yellow, or a magenta and a yellow dye are formed. Preferably a cyan dye-forming developer, a magenta dye-forming developer, and a yellow dye-forming developer are employed to form respectively cyan, magenta, and yellow dyes from the same coupler. In another embodiment a black dye forming developer is additionally employed. In yet another embodiment multiple cyan dye forming, magenta dye forming, and yellow dye forming developers can be individually employed to form a greater gamut of colors or to form colors at greater bit depth.

A cyan dye is a dye having a maximum absorption at between 580 and 700 nm, with preferably a maximum absorption between 590 and 680 nm, more preferably a peak absorption between 600 and 670 nm, and most preferably a peak absorption between 605 and 655 nm. A magenta dye is a dye having a maximum absorption at between 500 and 580 nm, with preferably a maximum absorption between 515 and 565 nm, more preferably a peak absorption between 520 and 560 nm, and most preferably a peak absorption between 525 and 555 nm. A yellow dye is a dye having a maximum absorption at between 400 and 500 nm, with preferably a maximum absorption between 410 and 480 nm, more preferably a peak absorption between 435 and 465 nm, and most preferably a peak absorption between 445 and 455 nm. The concentrations and amounts of the distinct developers and the multifunctional dye forming coupler will typically be chosen so as to enable the formation of dyes having a density at maximum absorption of at least 0.7, preferably a density of at least 1.0, more preferably a density of at least 1.3, and most preferably a density of at least 1.6. Further, the dyes will typically have a half height band width (HHWB) of between 70 and 170 nm in the region between 400 and 700 nm. Preferably, the HHWB will be less than 150 nm, more preferably less than 130 nm, and most preferably less than 115 nm. Additional details of preferred dye hues are described by McInerney et al in U.S. Pat. Nos. 5,679,139; 5,679,140; 5,679,141; and 5,679,142, the disclosures of which are incorporated by reference.

The multifunctional dye forming couplers useful in the invention can be functionally defined based on the color of the dye formed by specific color developers.

Thus a useful imaging member comprises a multifunctional dye that when reacted with the oxidized form of a developer of structure II:



wherein:

n is 0, 1, or 2;

A is OH or NR3R4;

Y is H, or a group that reacts before or during a coupling reaction to form H; when Y is a group that reacts before or during a coupling reaction to form H, then Y is preferably the moiety Q-R6 wherein:

R6 is H, alkyl, substituted alkyl, alkenyl, substituted alkenyl, alkynyl, substituted alkynyl, aryl, substituted aryl, heterocyclic or substituted heterocyclic, and Q is  $-SO_2-$ ,  $-SO-$ ,  $-SO_3-$ ,  $-CO-$ ,  $-COCO-$ ,  $-CO-O-$ ,  $-CO(NR7)-$ ,  $-COCO-O-$ ,  $-COCO-N(R7)-$ , or  $-SO_2-N(R7)-$ , where R7 is H or the groups described in R6; and

R1, R2, R3, and R4, which can be the same or different, are individually H, alkyl, substituted alkyl, alkenyl, substituted alkenyl, aryl, substituted aryl, halogen, cyano, alkoxy, substituted alkoxy, aryloxy, substituted aryloxy, amino, substituted amino, alkylcarbonamido, substituted alkylcarbonamido, arylcarbonamido, substituted arylcarbonamido,

alkylsulfonamido, arylsulfonamido, substituted alkylsulfonamido, substituted arylsulfonamido, or sulfamyl, or wherein at least two of R1, R2, R3, and R4 together further form a substituted or unsubstituted carbocyclic or heterocyclic ring structure; results in a magenta dye being formed.

Specific examples of magenta dye forming developers include but are not limited to the oxidized form of a color developer chosen from the group consisting of N,N-diethyl-p-phenylenediamine, 4-N,N-diethyl-2-methylphenylene diamine, 4-(N-ethyl-N-2-methanesulfonylaminoethyl)-2-methylphenylenediamine, 4-(N-ethyl-N-2-hydroxyethyl)-2-methylphenylenediamine, 4-N,N-diethyl-2-methanesulfonylaminoethylphenylenediamine, 4-(N-ethyl-N-2-methoxyethyl)-2-methylphenylenediamine, 4,5-dicyano-2-isopropylsulfonylhydrazinobenzene, and 4-amino-2,6-dichlorophenol. Preferred magenta dye forming developers can also be physically characterized as having an  $E_{1/2}$  at pH 11 more positive than 190 mV. The sign convention and method of measuring the oxidation-reduction potential or  $E_{1/2}$  of a developer is that described in *The Theory of the Photographic Process*, 4th ed., T. H. James, ed., Macmillan, New York, 1977, at pages 291-403, the disclosures of which are incorporated by reference. This reference is additionally cited for its disclosure of specific developers useful in the practice of this invention. Other useful developers and developer precursors are disclosed by Hunig et al, *Angew. Chem.*, 70, page 215-ff (1958), by Schmidt et al U.S. Pat. No. 2,424,256; Pelz et al U.S. Pat. No. 2,895,825; Wahl et al U.S. Pat. No. 2,892,714; Clarke et al U.S. Pat. Nos. 5,284,739 and 5,415,981; Takeuchi et al U.S. Pat. 5,667,945; and Nabeta U.S. Pat. 5,723,277, the disclosures of which are incorporated by reference.

Further, a useful imaging member comprises a multifunctional dye that when reacted with the oxidized form of a developer of structure III:



wherein n, A, Y, R1, and R2 are as defined above; results in a cyan dye being formed.

Specific examples of such cyan forming developers include but are not limited to the oxidized form of a color developer chosen from the group consisting of 4-N,N-diethyl-2-methyl-6-methoxyphenylenediamine, 4-N,N-diethyl-2,6-dimethylphenylenediamine, 4-(N-ethyl-N-2-methanesulfonylaminoethyl)-2,6-dimethylphenylenediamine, 4-(N-ethyl-N-2-hydroxyethyl)-2,6-dimethylphenylenediamine, 4-N,N-diethyl-2-methanesulfonylaminoethyl-6-methylphenylenediamine, 4-(N-ethyl-N-2-hydroxyethyl)-2-ethoxyphenylene diamine, and 4-(N-ethyl-N-2-methoxyethyl)-2,6-dimethylphenylenediamine. Preferred cyan dye forming developers can also be characterized in having an  $E_{1/2}$  at pH 11 less positive than 200 mV.

And further, a useful imaging member comprises a multifunctional dye that when reacted with the oxidized form of a developer of structure IV:



wherein n, A, Y, R1, and R2 are as defined above, results in a yellow dye being formed.

Preferred yellow dye forming developers can also be characterized in having an  $E_{1/2}$  at pH 11 more positive than 220 mV.

It is preferred to employ an oxidized form of a color developer of structure V:



wherein R5 is alkyl, substituted alkyl, alkenyl, substituted alkenyl, aryl, substituted aryl, substituted carbonyl, substi-

tuted carbamyl, substituted sulfonyl, substituted sulfamyl, heterocyclic, or substituted heterocyclic; Y is as defined above, and which results in a yellow dye being formed.

Specific examples of yellow dye forming developers include, but are not limited to, the oxidized form of a color developer chosen from the group consisting of 2-hydrazino-2-imidazoline, 4-hydrazinobenzoic acid, 2-hydrazinobenzoic acid, 4-hydrazinobenzenesulfonic acid, 9-hydrazinocridine, 2-hydrazinobenzothiazole, 1-hydrazinophthalazine, 2-hydrazinopyridine, 3-(hydrazinosulfonyl)benzoic acid, 3-hydrazinoquinoline, 1,3-diethyl-2-hydrazinobenzimidazole, 4-(N-ethyl, N-carbonamidomethyl)-phenylenediamine, and 4-morpholinophenylenediamine.

In one preferred embodiment, the partial structure  $-(CR_1=CR_2)_n-$  represents a substituted or unsubstituted phenyl moiety. When  $(CR_1=CR_2)_n$  represents an aromatic moiety, the moieties A—and —NHY are preferably in a para relationship, one to another.

In structures II, III, IV, and V, the word "substituted" at each occurrence represents any group other than H needed to satisfy the required valence which does not adversely affect the required properties. The word "substituted" preferably represents one or more of a linear or branched carbonaceous group which can be cyclic or acyclic, a heterocyclic group, an aromatic carbonaceous group, an arylalkyl group, a halogen atom, a cyano group, a nitro group, a ureido group, an ether group, an ester group, an amine group, an amide group, a thioether group, a thioester group, a sulfonyl group, or a sulfamyl group.

The developer structures described above are generally 2-electron equivalent developers.

The individual developers or developer precursors are generally applied in an imagewise fashion to the member from a developer solution. The developer solution can be aqueous or non-aqueous. When the developer solution is an aqueous solution, it can contain pH adjusting agents and developer or developer precursor stabilizers. The pH of the solution can be adjusted for optimum cross-oxidation as known in the art, or it can be adjusted for optimum storage stability. In the latter case, the pH of the member can be adjusted separately. The pH adjustment can employ a buffer consisting of an organic or inorganic acid or base and/or a salt thereof. Useful examples include phosphoric acid and salts of phosphates, sulfuric acid and salts of sulfate, citric acid and salts of citrate, boric acid and salts of borate or metaborate, acetic acid and salts of acetate, salts of carbonate, amines and amine salts, urea derivatives and their salts, and ammonium hydroxide or mixtures thereof. Developer stabilizers can be present in the developer solution as known in the art. Additionally, the developer can be supplied in a blocked form which unblocks and releases the developer before or during its oxidation or a coupling reaction. When the developer is supplied in its blocked form, that form can be any blocked form known in the art that unlocks under the conditions encountered in practicing the invention. In addition to the blocking groups already described, developers that are deactivated as sulfate, hydrochloride, sulfite and p-toluenesulfonate salts, or are deactivated as metal complexes, all as known in the art, are specifically contemplated. The concentration of the developer or developer precursor in the developer solution will be that needed to enable adequate density formation to be attained on applying the developer solution to the member. Preferably, the developer or developer precursor will be present in the developer solution at a concentration between about 2 and 100 g/L. It is more preferred that the developer or developer precursor will be present in the developer solution at a concentration between about 10 and 50 g/L.

An auxiliary developer or electron transfer agent as known in the art can additionally be present in the member

during image formation to aid the catalytic center in its interaction with the developer and the oxidant. The auxiliary developer or electron transfer agent can be incorporated in the member at manufacture, or it can be added to the member before or during image formation. Additionally, oxidized developer scavengers and competing developers can be added to the member before, during, or after image formation to aid in the stability, color reproduction and colorfulness of the member and the produced images. These and other useful agents are described, *inter alia*, at *Research Disclosure*, Item 37038, (1995), Section III, and at *Research Disclosure*, Item 38957, (1996), Section XIX.

The developer can be imagewise applied to the imaging member in any manner known in the art. In one embodiment, the developer can be thermally ablated in an imagewise manner from a donor sheet or ribbon to the imaging member. In a preferred embodiment, the developer is carried in a developer solution, and that solution is imagewise applied to the imaging member. A preferred method of imagewise application of developer solution is by the technique colloquially known as "ink jet". In ink jet application, tiny droplets of developer solution are projected directly onto the imaging member without physical contact between the projecting device and the imaging member. The placement of each drop on the imaging member is controlled electronically. The projecting device is called a printhead. Imaging is accomplished by moving the printhead across the imaging member, or by moving the imaging member across the printhead. One or more printheads, each driving one or more projected streams, is known in the art and is specifically contemplated for use in the invention.

Different types of ink jet projection are known. Two major forms of ink jet projection are "drop-on-demand" projection and "continuous jet" projection. Continuous jet projection is characterized by pressure-projecting developer solution through a nozzle to generate drops of developer solution directed in a continuous stream towards the imaging member while passing through an imagewise modulated solution deflection system thereby allowing developer solution droplets of the stream to deposit imagewise on the imaging member. Drop-on-demand or impulse ink jet differs from continuous ink jet in that the developer solution supply is maintained at or near atmospheric pressure. A drop is ejected from a nozzle only on demand when controlled excitation coming from pressure generated by a piezoelectric element or from pressure generated by local electrothermal evaporation of liquid (thermal bubble jet) is applied to a developer filled channel ending in a nozzle. Acoustic, microfluidic, and electrostatic driven drop-on-demand techniques are also known. These technologies, as they apply to the application of inks, are described in detail by J. L. Johnson, *Principles of Non-Impact Printing*, Palatino Press, Irvine, Calif. (1986), and in *Nebblette's Imaging Processes and Materials*, Eighth Edition, J. Sturges Ed. Van Nostrand, New York, (1989). Both drop-on-demand and continuous developer solution applications are particularly contemplated as imagewise solution application techniques to be employed in the practice of this invention.

In employing ink jet application of developer solution, any size and any number of drops can be applied to a specific area of the imaging member to best form the desired image. The size and the number of drops of solution are controlled by the specific design of the printhead and by the electronic driver of the printhead. The electronic driver of the printhead, in turn, is controlled by the digital characteristics of the digitized image being printed. The individual drops will typically be between 1 and 50 picoliters in volume. The individual drops will preferably be less than 30 picoliters, and more preferably less than 10 picoliters in volume. The use of smaller drops is preferred since the imaging member is less wetted and since this better allows the application of

multiple drops to a particular area of the imaging member. Any individual area of the imaging member can receive between 1 and 50 drops. In a preferred embodiment, any individual area of the imaging member will receive at least 3 drops, one from each of three printheads delivering distinct developer solutions which enable the formation of cyan, magenta, and yellow dyes. It is more preferred to employ four printheads to deliver distinct developer solutions, thereby enabling the formation of cyan, magenta, yellow, and black dyes. In another embodiment, an imaging apparatus can be configured to employ distinct printheads to deliver developer solutions according to this invention and to also deliver soluble inks or particulate inks as known in the art. This latter mode is particularly preferred when a black image deposit is desired. In yet another embodiment, six solution delivery systems, each supplying a distinct developer, developer mixture, or ink, can be employed to independently form two cyan images differing in density or hue, two magenta images differing in density or hue, a yellow image, and a black image at the imaging member.

The imaging member can be heated during or after application of the developer. This heating has many useful functions including, but not limited to, driving the oxidation and reduction reactions to completion, driving the coupling reaction to completion, and drying the imaging member.

Temperatures in excess of room temperature are generally preferred. When the imaging member is heated, it will generally be heated to a temperature of at least 35° C. It will preferably be heated to a temperature of at least 80° C., more preferably it will be heated to a temperature of at least 100° C., and most preferably, it will be heated to a temperature of at least 110° C. When the imaging member is heated, it will generally be heated to a temperature of up to 200° C. It will preferably be heated to a temperature of up to 160° C., and more preferably be heated to a temperature of up to 140° C. The imaging member can be held at an elevated temperature

for whatever time is required to achieve adequate density formation. Heating times of up to 120 seconds are generally adequate, while heating times of up to 60 seconds are preferred, heating times of up to 30 seconds are more preferred, and heating times of 10 seconds are most preferred.

Most generally, higher temperatures enable the use of shorter heating times as is well known in the chemical arts. Any known apparatus suitable for heating can be employed for this purpose.

The following examples illustrate the practice of this invention. They are not intended to be exhaustive of all possible variations of the invention. Parts and percentages are by weight unless otherwise indicated.

## EXAMPLES

### Example 1

An imaging layer was prepared which contained 2.37 g/m<sup>2</sup> of silver behenate, 0.43 g/m<sup>2</sup> of coupler A-1, 0.080 g/m<sup>2</sup> of hardening agent bis(vinylsulfonyl)methane, and 4.74 g/m<sup>2</sup> of gelatin. This image receiving layer was coated on a reflection support.

A cyan dye-forming developer solution, Developer Solution A, was prepared which contained 0.2 g of 4-N,N-diethyl-2,6-dimethylphenylenediamine, in 5 g of distilled water and 5 g of methanol. A magenta dye-forming developer solution, Developer Solution B, was prepared which contained 0.2 g of 4-(N-ethyl-N-2-hydroxyethyl)-2-methylphenylenediamine in 5 g of distilled water and 5 g of methanol. A yellow dye-forming developer solution, Developer Solution C, was prepared which contained 0.2 g of 2-hydrzinobenzothiazole in 5 g of distilled water and 5 g of methanol. The reservoirs of ink jet printer cartridges for an HP Deskjet 855Cxi printer were individually filled with the

cyan, magenta, and yellow dye-forming Developer Solutions A, B, and C. Using the ink jet printer, image patterns of the three Developer Solutions were applied to the image receiving layer. The coating was uniformly heated for 5 seconds at 130° C. Cyan dye formed in the regions where the cyan dye-forming Developer Solution was applied. Magenta dye formed in the regions where the magenta dye-forming Developer Solution was applied. Yellow dye formed in the regions where the yellow dye-forming Developer Solution was applied. Status A reflection densities are shown in Table 2 for the three color patches. The results in Table 2 illustrate that the combination of dyes formed provide both high optical densities and span a large color gamut.

TABLE 2

| Color patch | Red Density | Green Density | Blue Density |
|-------------|-------------|---------------|--------------|
| A           | 1.462       | 0.842         | 0.703        |
| B           | 0.699       | 1.962         | 1.027        |
| C           | 0.923       | 1.616         | 1.853        |

To measure the waterfastness of the image dyes, the optical density corresponding to peak absorption for the color patches was measured before and after immersing the paper in distilled water for 5 minutes and drying the coating. The waterfastness was calculated as the percentage of the initial optical density retained during this treatment. That is, a waterfastness value of 100 indicates the optical density did not change, and a value of 0 indicates that all of the image dye was removed from the image receiving layer during the waterfastness test. Table 3 shows the dyes formed are completely waterfast.

TABLE 3

| Color patch | Waterfastness |
|-------------|---------------|
| Cyan        | 101           |
| Magenta     | 102           |
| Yellow      | 102           |

## Comparative Example 2

To further illustrate the advantage in waterfastness obtained by practicing the current invention, the cyan, magenta, and yellow inks in an HP51641 A color ink jet cartridge were applied to a photo quality ink jet paper to generate cyan, magenta, and yellow color patches. The waterfastness of these image dyes was measured as described above, and results are shown in Table 4. The waterfastness was poor for all three HP dyes, with only between 2 and 40% of the initial optical density remaining. It is clear by comparing the waterfastness values in Tables 3 and 4 that practice of the current invention provides an output material with excellent waterfastness.

TABLE 4

| Color patch | Comparison, Optical Density HP inks | Comparison, Waterfastness HP inks |
|-------------|-------------------------------------|-----------------------------------|
| Cyan        | 1.16                                | 45                                |
| Magenta     | 1.23                                | 20                                |
| Yellow      | 1.16                                | 2                                 |

The invention has been described in detail with particular reference to certain preferred embodiments thereof, but it will be understood that variations and modifications can be effected within the spirit and scope of the invention.

What is claimed is:

- An imaging member comprising a support and at least one light insensitive layer comprising an oxidant and a multifunctional dye forming coupler.
- The imaging member of claim 1 wherein said oxidant is a metal salt that forms a metallic deposit on reduction.
- The imaging member of claim 2 wherein said metal salt is selected from the group consisting of salts of vanadium, chromium, manganese, iron, cobalt, nickel, copper, niobium, molybdenum, ruthenium, rhodium, palladium, silver, cadmium, tantalum, tungsten, rhenium, osmium, iridium, platinum, and gold.
- The imaging member of claim 3 wherein said metal salt is selected from the group consisting of the reducible silver fatty acid salts, the reducible salts of silver alkylacetylide, the reducible salts of silver arylacetylide, the reducible salts of silver alkylamines, the reducible salts of silver arylamines, the reducible salts of heterocyclic silver mercaptides, and the reducible salts of heterocyclic silver thiones.
- The imaging member of claim 4 wherein said metal salt comprises a reducible silver fatty acid salt.
- The imaging member of claim 2 wherein said metal salt comprises silver behenate.
- The imaging member of claim 2 wherein said silver salt comprises silver benzotriazole.
- The imaging member of claim 2 wherein said silver salt comprises silver acetylide.
- The imaging member of claim 2 wherein said silver salt comprises silver 5-amino-2-benzylthiotaiazole.
- The imaging member of claim 1 wherein said oxidant is a metal salt forms a metal salt of lower oxidation state on reduction.
- The imaging member of claim 1 wherein said multifunctional dye-forming coupler is a 2-equivalent coupler.
- The imaging member of claim 1 wherein said oxidant is a metal salt in a particulate form and has a particle size of between 0.1  $\mu$ m and 30  $\mu$ m.
- The imaging member of claim 1 wherein said oxidant is a non-metallic oxidant.
- The imaging member of claim 13 wherein said non-metallic oxidant is chosen from the group consisting of the hydrogen, alkali and alkali earth salts of persulfate, peroxide, perborate, and percarbonate, oxygen, and the related perhalogen oxidants such as hydrogen, alkali, and alkali earth salts of chlorate, bromate, iodate, perchlorate, perborate, and metaperiodate.
- The imaging member of claim 1 further comprising an oxidation catalyst.
- The imaging member of claim 1 wherein said support comprises a reflective support.
- The imaging member of claim 1 wherein said support comprises a transparent support.
- The imaging member of claim 1 wherein said multifunctional dye-forming coupler comprises a coupler of the following structure I:



(I)

60 wherein:

- C is a carbon atom at which coupling occurs;  
 L represents a hydrogen atom or a leaving group covalently bound to C and which is displaced on coupling;  
 H is an acidic hydrogen atom serving to direct coupling to C and which is covalently bound to C directly or by conjugation; and

Z represents the remainder of the atoms of the coupler, in cyclic or acyclic form, which together provide sufficient electron withdrawal to render H acidic and together provide sufficient ballast function to render the dye formed from the coupler immobile.

19. The imaging member of claim 1 wherein said coupler is chosen from the group consisting of a pyrazole, a pyrazolone, a pyrazolotriazole, pyrazolotetrazole, a 2-acylamino-1-naphthol and a cyanoacetate coupler.

20. The imaging member of claim 1 wherein said coupler is chosen from the group consisting of couplers A-1 through A-14, having structures according to the specification.

21. The imaging member of claim 1 wherein said multi-functional dye-forming coupler will form different colors when it reacts with different oxidized developers.

22. The imaging member of claim 1 wherein said multi-functional dye-forming coupler comprises a coupler that when reacted with the oxidized form of a developer of structure II:

A—(CR1==CR2)<sub>n</sub>—NHY

(II) 20

wherein:

n is 0, 1, or 2;

A is OH or NR3R4;

Y is H, or a group that reacts before or during a coupling reaction to form H; and

R1, R2, R3, and R4, which can be the same or different, are individually H, alkyl, substituted alkyl, alkenyl, substituted alkenyl, aryl, substituted aryl, halogen, cyano, alkoxy, substituted alkoxy, aryloxy, substituted aryloxy, amino, substituted amino, alkylcarbonamido, substituted alkylcarbonamido, arylcarbonamido, substituted arylcarbonamido, alkylsulfonamido, arylsulfonamido, substituted alkylsulfonamido, substituted arylsulfonamido, or sulfamyl or wherein at least two of R1, R2, R3, and R4 together further form a substituted or unsubstituted carbocyclic or heterocyclic ring structure;

results in a magenta dye being formed.

23. The imaging member of claim 1 wherein said multi-functional dye-forming coupler comprises a coupler that when reacted with the oxidized form of a developer of structure III:

A—(CR1==CR2)<sub>n</sub>—NHY

(III) 45

wherein:

n is 0, 1, or 2;

A is OH or NR3R4;

Y is H, or a group that reacts before or during a coupling reaction to form H; and

R1, R2, R3, and R4, which can be the same or different, are individually H, alkyl, substituted alkyl, alkenyl, substituted alkenyl, aryl, substituted aryl, halogen, cyano, alkoxy, substituted alkoxy, aryloxy, substituted aryloxy, amino, substituted amino, alkylcarbonamido, substituted alkylcarbonamido, arylcarbonamido, substituted arylcarbonamido, alkylsulfonamido, arylsulfonamido, substituted alkylsulfonamido, substituted arylsulfonamido, or sulfamyl or wherein at least two of R1, R2, R3, and R4 together further form a substituted or unsubstituted carbocyclic or heterocyclic ring structure;

results in a cyan dye being formed.

24. The imaging member of claim 1 wherein said multi-functional dye-forming coupler comprises a coupler that

when reacted with the oxidized form of a developer of structure IV:

A—(CR1==CR2)<sub>n</sub>—NHY (IV)

5 wherein:

n is 0, 1, or 2;

A is OH or NR3R4;

Y is H or a group that reacts before or during a coupling reaction to form H; and

R1, R2, R3, and R4, which can be the same or different, are individually H, alkyl, substituted alkyl, alkenyl, substituted alkenyl, aryl, substituted aryl, halogen, cyano, alkoxy, substituted alkoxy, aryloxy, substituted aryloxy, amino, substituted amino, alkylcarbonamido, substituted alkylcarbonamido, arylcarbonamido, substituted arylcarbonamido, alkylsulfonamido, arylsulfonamido, substituted alkylsulfonamido, substituted arylsulfonamido, or sulfamyl or wherein at least two of R1, R2, R3, and R4 together further form a substituted or unsubstituted carbocyclic or heterocyclic ring structure;

results in a yellow dye being formed.

25. The imaging member of claim 1 wherein said multi-functional dye-forming coupler comprises a coupler that when reacted with the oxidized form of a color developer chosen from the group consisting of N,N-diethylphenylenediamine, 4-N,N-diethyl-2-methylphenylenediamine, 4-(N-ethyl-1-N-2-methanesulfonylaminoethyl)-2-methylphenylenediamine, 4-(N-ethyl-N-2-hydroxyethyl)-2-methylphenylenediamine, 4-N,N-diethyl-2-methanesulfonylaminoethylphenylenediamine, 4-(N-ethyl-N-2-methoxyethyl)-2-methylphenylenediamine, and 4-amino-3,5-dichlorophenol;

results in a magenta dye being formed.

26. The imaging member of claim 1 wherein said multi-functional dye-forming coupler comprises a coupler that when reacted with the oxidized form of a color developer chosen from the group consisting of 4-N,N-diethyl-2-methyl-6-methoxyphenylenediamine, 4-N,N-diethyl-2,6-dimethylphenylenediamine, 4-(N-ethyl-1-N-2-methanesulfonylaminoethyl)-2,6-dimethylphenylenediamine, 4-(N-ethyl-N-2-hydroxyethyl)-2,6-dimethylphenylenediamine, 4-N,N-diethyl-2-methanesulfonylaminoethyl-6-methylphenylenediamine hydrochloride, 4-(N-ethyl-N-2-hydroxyethyl)-2-ethoxyphenylenediamine, and 4-(N-ethyl-N-2-methoxyethyl)-2,6-dimethylphenylenediamine,

results in a cyan dye being formed.

27. The imaging member of claim 1 wherein said multi-functional dye-forming coupler comprises a coupler that when reacted with the oxidized form of a color developer of structure V:

R5-HN—NHY (V)

wherein R5 is alkyl, substituted alkyl, alkenyl, substituted alkenyl, aryl, substituted aryl, substituted carbonyl, substituted carbamyl, substituted sulfonyl, substituted sulfamyl, heterocyclic or substituted heterocyclic; and Y is H, or a group that reacts before or during a coupling reaction to form H;

results in a yellow dye being formed.

28. The imaging member of claim 1 wherein said multi-functional dye-forming coupler comprises a coupler that when reacted with the oxidized form of a color developer chosen from the group consisting of 2-hydrazino-2-imidazoline, 4-hydrazinobenzoic acid, 2-hydrazinobenzoic acid, 4-hydrazinobenzenesulfonic acid, 9-hydrazinoacridine, 2-hydrazinobenzothiazole,

1-hydrazinophthalazine, 2-hydrazinopyridine, 3-(hydrazinosulfonyl)benzoic acid, 3-hydrazinoquinoline, 1,3-diethyl-2-hydrazinobenzimidazole, 4-(N-ethyl, N-carbonamidomethyl)-phenylenediamine, and 4-morpholinophenylenediamine;

5 results in a yellow dye being formed.

29. The imaging member of claim 1 wherein the molar ratio of oxidant, to dye-forming coupler, is between 1.8:1 and 6:1.

30. A method of imaging comprising providing an imaging member comprising a support and at least one light insensitive layer comprising an oxidant and multifunctional dye-forming coupler, imagewise applying a first developer solution that will react with said oxidant and with said multifunctional dye-forming coupler, imagewise applying a second developer solution that will react with said oxidant and with said multifunctional dye-forming coupler, wherein said first developer solution and said second developer solution produce different colors.

31. The method of claim 30 wherein said oxidant is a 20 metal salt that forms a metallic deposit on reduction.

32. The method of claim 31 wherein said metal salt is selected from the group consisting of salts of vanadium, chromium, manganese, iron, cobalt, nickel, copper, niobium, molybdenum, ruthenium, rhodium, palladium, silver, cadmium, tantalum, tungsten, rhenium, osmium, iridium, platinum, and gold.

33. The method of claim 32 wherein said metal salt is selected from the group consisting of the reducible silver fatty acid salts, the reducible salts of silver alkylacetylide, the reducible salts of silver arylacetylide, the reducible salts of silver alkylamines, the reducible salts of silver arylamines, the reducible salts of heterocyclic silver mercaptides, and the reducible salts of heterocyclic silver thiones.

34. The method of claim 30 wherein said oxidant is a metal salt forms a metal salt of lower oxidation state on reduction.

35. The method of claim 34 wherein said metal salt is selected from the group consisting of the salts of vanadium, chromium, manganese, iron, cobalt, nickel, copper, niobium, molybdenum, ruthenium, rhodium, palladium, silver, cadmium, tantalum, tungsten, rhenium, osmium, iridium, platinum, and gold.

36. The method of claim 30 wherein said oxidant is a 45 metal salt in a particulate form and has a particle size between 0.1  $\mu\text{m}$  and 30  $\mu\text{m}$ .

37. The method of claim 30 wherein said oxidant is a non-metallic oxidant.

38. The method of claim 37 wherein said non-metallic oxidant is chosen from the group consisting of the hydrogen, alkali and alkali earth salts of persulfate, peroxide, perborate, and percarbonate, oxygen, and the related perhalogens oxidants bromate, iodate, perchlorate, perbromate, and metaperiodate.

39. The method of claim 38 wherein said related perhalogens oxidants are chosen from the group consisting of hydrogen, alkali and alkali earth salts of chlorate, bromate, iodate, perchlorate, perbromate and metaperiodate.

40. The method of claim 30 further comprising an oxidation catalyst.

41. The method of claim 30 wherein said support comprises a reflective support.

42. The method of claim 30 wherein said support comprises a transparent support.

43. The method of claim 30 wherein said multifunctional dye-forming coupler comprises a coupler of the following structure I:



(I)

10 wherein:

C is a carbon atom at which coupling occurs;

L represents a hydrogen atom or a leaving group covalently bound to C and which is displaced on coupling;

H is an acidic hydrogen atom serving to direct coupling to C and which is covalently bound to C directly or by conjugation; and

Z represents the remainder of the atoms of the coupler, in cyclic or acyclic form, which together provide sufficient electron withdrawal to render H acidic and together provide sufficient ballast function to render the dye formed from the coupler immobile.

44. The method of claim 30 wherein said coupler is chosen from the group consisting of a pyrazole, a pyrazolone, a pyrazolotriazole, pyrazolotetrazole, a 2-acylamino-1-naphthol, and a cyanoacetate coupler.

45. The method of claim 30 wherein said oxidant is a metal salt in a particulate form and has a particle size of up to about 5  $\mu\text{m}$ .

46. The method of claim 30 wherein said multifunctional dye-forming coupler will form different colors when it reacts with the oxidized form of different developers.

47. The method of claim 30 wherein said multifunctional dye-forming coupler comprises a coupler that when reacted with the oxidized form of a developer of structure II:



wherein:

n is 0, 1, or 2;

A is OH or NR3R4;

Y is H, or a group that reacts before or during a coupling reaction to form H; and

R1, R2, R3, and R4, which can be the same or different, are individually H, alkyl, substituted alkyl, alkenyl, substituted alkenyl, aryl, substituted aryl, halogen, cyano, alkoxy, substituted alkoxy, aryloxy, substituted aryloxy, amino, substituted amino, alkylcarbonamido, substituted alkylcarbonamido, arylcarbonamido, substituted arylcarbonamido, alkylsulfonamido, arylsulfonamido, substituted alkylsulfonamido, substituted arylsulfonamido, or sulfamyl or wherein at least two of R1, R2, R3, and R4 together further form a substituted or unsubstituted carbocyclic or heterocyclic ring structure;

55 results in a magenta dye being formed.

48. The method of claim 30 wherein said multifunctional dye-forming coupler forming coupler comprises a coupler that when reacted with the oxidized form of a developer of structure III:



wherein:

n is 0, 1, or 2;

A is OH or NR3R4;

Y is H or a group that reacts before or during a coupling reaction to form H; and

R1, R2, R3, and R4, which can be the same or different, are individually H, alkyl, substituted alkyl, alkenyl, substituted alkenyl, aryl, substituted aryl, halogen, cyano, alkoxy, substituted alkoxy, aryloxy, substituted aryloxy, amino, substituted amino, alkylcarbonamido, substituted alkylcarbonamido, arylcarbonamido, substituted arylcarbonamido, alkylsulfonamido, arylsulfonamido, substituted alkylsulfonamido, substituted arylsulfonamido, or sulfamyl or wherein at least two of R1, R2, R3, and R4 together further form a substituted or unsubstituted carbocyclic or heterocyclic ring structure;

results in a cyan dye being formed.

49. The method of claim 30 wherein said multifunctional dye-forming coupler comprises a coupler that when reacted with the oxidized form of a developer of structure IV:



wherein:

n is 0, 1, or 2;

A is OH or NR3R4;

Y is H, or a group that reacts before or during a coupling reaction to form H; and

R1, R2, R3, and R4, which can be the same or different, are individually H, alkyl, substituted alkyl, alkenyl, substituted alkenyl, aryl, substituted aryl, halogen, cyano, alkoxy, substituted alkoxy, aryloxy, substituted aryloxy, amino, substituted amino, alkylcarbonamido, substituted alkylcarbonamido, arylcarbonamido, substituted arylcarbonamido, alkylsulfonamido, arylsulfonamido, substituted alkylsulfonamido, substituted arylsulfonamido, or sulfamyl or wherein at least two of R1, R2, R3 and R4 together further form a substituted or unsubstituted carbocyclic or heterocyclic ring structure;

results in a yellow dye being formed.

50. The method of claim 30 wherein said multifunctional dye-forming coupler comprises a coupler that when reacted with the oxidized form of a color developer chosen from the group consisting of N,N-diethyl-p-phenylenediamine, 4-N, N-diethyl-2-methylphenylenediamine, 4-(N-ethyl-N-2-methanesulfonylaminoethyl)-2-methylphenylenediamine, 4-(N-ethyl-N-2-hydroxyethyl)-2-methylphenylenediamine, 4-N,N-diethyl-2-methanesulfonylaminoethylphenylenediamine hydrochloride, 4-(N-ethyl-N-2-methoxyethyl)-2-methylphenylenediamine, and 4-amino-3,5-dichlorophenol; results in a magenta dye being formed.

51. The method of claim 30 wherein said multifunctional dye-forming coupler comprises a coupler that when reacted with the oxidized form of a color developer chosen from the group consisting of 4-N,N-diethyl-2-methyl-6-methoxyphenylenediamine, 4-N,N-diethyl-2,6-dimethylphenylenediamine, 4-(N-ethyl-N-2-methanesulfonylaminoethyl)-2,6-dimethylphenylenediamine, 4-(N-ethyl-N-2-hydroxyethyl)-2,6-dimethylphenylenediamine, 4-N,N-diethyl-2-methanesulfonylaminoethyl-6-methylphenylenediamine hydrochloride, 4-(N-ethyl-N-2-hydroxyethyl)-2-ethoxyphenylenediamine, and 4-(N-ethyl-N-2-methoxyethyl)-2,6-dimethylphenylenediamine;

results in a cyan dye being formed.

52. The method of claim 30 wherein said multifunctional dye-forming coupler comprises a coupler that when reacted with the oxidized form of a color developer chosen from the group consisting of 2-hydrazino-2-imidazoline, 4-hydrazinobenzoic acid, 2-hydrazinobenzoic acid, 4-hydrazinobenzenesulfonic acid, 9-hydrazinoacridine, 2-hydrazinobenzothiazole, 1-hydrazinophthalazine, 2-hydrazinopyridine, 3-(hydrazinosulfonyl)benzoic acid, 3-hydrazinoquinoline, 1,3-diethyl-2-hydrazinobenzimidazole, 4-(N-ethyl-N-carbonamidomethyl)-phenylenediamine, and 4-morpholinophenylenediamine;

results in a yellow dye being formed.

53. The method of claim 30 wherein said multifunctional dye-forming coupler comprises a coupler that when reacted with the oxidized form of a color developer of structure V:



wherein R5 is alkyl, substituted alkyl, alkenyl, substituted alkenyl, aryl, substituted aryl, substituted carbonyl, substituted carbamyl, substituted sulfonyl, substituted sulfamyl, heterocyclic or substituted heterocyclic; and Y is H, or a group that reacts before or during a coupling reaction to form H;

results in a yellow dye being formed.

54. The method of claim 30 wherein said at least one of said first developer and said second developer is supplied in a blocked form.

55. The method of claim 54 wherein said imagewise application of said second developer solution and the imagewise application of a third developer solution results in cyan and yellow dyes being formed.

56. The method of claim 30 wherein imagewise application of developer solutions is by ink jet.

57. The method of claim 30 wherein imagewise application of developer solutions is carried out with separate application of oxidant and developing agent.

58. The method of claim 30 further comprising the imagewise application of a third developer solution that will react with said multifunctional dye-forming coupler.

59. The method of claim 30 wherein the imagewise application of said first developer solution results in a magenta dye being formed.

60. The method of claim 30 wherein said different colors differ in peak absorption wavelength by at least 50 nanometers.

61. The method of claim 30 comprising the step of heating said imaging member.

62. The method of claim 30 wherein the molar ratio of oxidant to dye forming coupler is between 1.8:1 and 6:1.

63. A method of imaging comprising providing an imaging member comprising a support and at least one light insensitive layer comprising a multifunctional dye-forming coupler, imagewise applying an oxidant, applying a first developer solution that will react with said oxidant and said multifunctional dye-forming coupler, imagewise applying a second developer solution that will react with said oxidant and said multifunctional dye-forming coupler, wherein said first developer solution and said second developer solution produce different colors.

64. The method of claim 63 comprising the step of heating said imaging member.

65. The method of claim 63 wherein said oxidant comprises silver behenate.

UNITED STATES PATENT AND TRADEMARK OFFICE  
**CERTIFICATE OF CORRECTION**

PATENT NO. : 6,440,896 B1  
DATED : August 27, 2002  
INVENTOR(S) : Richard P. Szajewski et al.

Page 1 of 1

It is certified that error appears in the above-identified patent and that said Letters Patent is hereby corrected as shown below:

Column 27,

Lines 54 and 55, delete "bromate, iodate, perchlorate, perbromate, and metaperiodate"

Column 28,

Line 58, delete "forming coupler" (second occurrence)

Signed and Sealed this

Fourth Day of February, 2003



JAMES E. ROGAN  
*Director of the United States Patent and Trademark Office*